

## UNITED STATES PATENT OFFICE

ADOLF KLINKENBERG, OF WITTBERG, NEAR HERDECKE, GERMANY, ASSIGNOR TO  
THE FIRM VEREINIGTE STAHLWERKE AKTIENGESELLSCHAFT, OF DUSSELDORF,  
GERMANY

## STEEL HAVING A HIGH YIELD POINT AND A GOOD NOTCH TOUGHNESS

No Drawing. Application filed January 29, 1931, Serial No. 512,194, and in Germany January 8, 1930.

As is well known the physical properties of steel are influenced by phosphorus to quite a considerable degree in such a way that by an addition of about 0.1% of phosphorus the 5 yield point as well as the tensile strength are considerably increased, the capability of changing the form, particularly the notch toughness very considerably decreased. Therefore, phosphorus as an unquestioned 10 generator of cold-shortness belongs to the undesirable elements in the metallurgy of iron and generally speaking is held in decidedly low repute (cf. Oberhoffer: Das technische Eisen, page 206). It is for this reason that 15 the alloying value of phosphorus is made use of to a very limited extent only in spite of the influence of phosphorus on the yield point and tensile strength that in itself is a favorable one. Thus for parts of minor importance, such as pressed nuts, bicycle parts etc. phosphorus bearing steels are used to a 20 limited extent since they have a clean surface after cold-working. In a similar way the action of phosphorus is utilized for the purpose of increasing the capability of being worked 25 by cutting tools of the free cutting steel. Thus the use of phosphorus bearing steels is relatively limited to fields wherein the stresses are small and at the same time the breaking 30 safety factor is of minor importance. For use in higher stressed structural material, for example in the construction of bridges, vehicles or machines the phosphorus content of the steel has heretofore been kept relatively 35 low considering the danger of cold-shortness. Thus in the standard steels the phosphorus content is limited to a maximum amount of 0.06%.

According to the invention one succeeds in 40 producing phosphorus bearing steels having a high yield point and tensile strength without causing the heretofore unavoidable great reduction in toughness to take place as a result of the phosphorus content by alloying a 45 certain percentage of copper with the phos-

phorus bearing steels, which are poor in carbon. It is true that with increasing tensile strength a corresponding decrease in the strain values takes place, but the notch toughness of the phosphorus-copper steels which 50 are the subject of the invention suffices for the practical purposes of the erection of large steel structures.

The carbon and phosphorus contents have a certain reciprocal action and this is the 55 reason why it is to be preferred to fix the upper limit of the carbon content at about 0.3%. Preferably the phosphorus content is added already in starting the melt by suitably composing the charge and is maintained, particularly in the basic Bessemer process, by intercepting the melt. In a similar way the copper content may also originate from the charge or it may be added to the finished melt in solid or liquid form. The upper limit of 60 the copper content is about 1%. Furthermore it has proved advantageous to deoxidize the melt in known manner for the purpose of avoiding segregation by means of the usual deoxidizers, such as silicon, manganese or 65 aluminum.

By combining suitable proportions of phosphorus and copper new steels are produced for a great variety of uses in connection with the erection of large steel structures. In 70 order to illustrate the excellent tensile properties of such steels the following examples are given:

(1) A steel of the following composition: 75 0.10% C, 0.1% Si, 0.50% Mn, 0.14% P, 0.05% S, 0.64% Cu, had the following physical properties:

| Yield point<br>kg./mm. <sup>2</sup> | Tensile strength<br>kg./mm. <sup>2</sup> | Extensio<br>n<br>δ 10<br>per<br>cent | Con-<br>trac-<br>tion<br>per<br>cent | Yield point<br>Tensile strength<br>per cent<br>×100 |       | Notch<br>toughness<br>mkg./cm. <sup>2</sup> |
|-------------------------------------|------------------------------------------|--------------------------------------|--------------------------------------|-----------------------------------------------------|-------|---------------------------------------------|
|                                     |                                          |                                      |                                      | 77                                                  | 10-13 |                                             |
| 39.5                                | 51.3                                     | 23.5                                 | 50                                   |                                                     |       |                                             |

85

90

(2) A steel of the same composition yet with 0.22% P had the following physical properties:

| 5 | Yield point<br>kg./mm. <sup>2</sup> | Break-<br>ing stress<br>kg./mm. <sup>2</sup> | Exten-<br>sion<br>$\delta$ 10<br>per<br>cent | Con-<br>trac-<br>tion<br>per<br>cent | Yield point<br>Tensile strength $\times 100$<br>per cent | Notch<br>toughness<br>mkg./cm. <sup>2</sup> |
|---|-------------------------------------|----------------------------------------------|----------------------------------------------|--------------------------------------|----------------------------------------------------------|---------------------------------------------|
|   | 10                                  | 44.5                                         | 53.5                                         | 25                                   | 55                                                       | 83                                          |

15 The phosphorus-copper steels, apart from good static properties have also a high fatigue limit, thus with the steel of Example (1) a fatigue limit of  $\pm 34$  kg./mm.<sup>2</sup> has been ascertained on the rotating beam testing machine. Furthermore, by increasing the phosphorus content the resistance to wear is practically considerably increased and the tendency to rust decreased.

20 20 What I claim and desire to secure by Letters Patent of the United States is:

25 1. A steel having a high yield point and a good notch toughness, a low carbon content from about 0.1% to 0.3%, a small amount of sulphur not exceeding 0.05%, a phosphorus content ranging between 0.1 and 0.4% and a copper content of between 0.1 and 1% and the remainder substantially iron.

30 2. A steel having a yield point ranging from 39.5 to 44.5 kg. per sq. mm. and a notch toughness ranging from 10 to 13 mkg. per sq. cm., a carbon content from about 0.01% to 0.3%, a phosphorus content ranging from 0.1 to 0.4%, a small amount of sulphur not exceeding 0.05% and a copper content of 0.1 to 1% and the remainder substantially iron.

35 3. A steel of the following composition: 0.1% carbon, 0.1% silicon, 0.5% manganese, 40 0.14% phosphorus, 0.05% sulphur, 0.64% copper and the remainder substantially iron.

In testimony whereof I affix my signature.  
ADOLF KLINKENBERG.

45

50

55

60

65